

July 9, 1940.

C. T. GREENIDGE

2,206,888

METHOD OF CONTINUOUS METAL CASTING

Filed Nov. 8, 1938



ATTORNEYS

## UNITED STATES PATENT OFFICE

2,206,888

## METHOD OF CONTINUOUS METAL CASTING

Charles T. Greenidge, Columbus, Ohio, assignor,  
by mesne assignments, to Edward R. Williams  
and Julia Lee Cox Williams, as joint tenants  
with right of survivorship

Application November 8, 1938, Serial No. 239,490

6 Claims. (Cl. 22—200.1)

This application relates to the continuous casting of metal in a definite shape and form and is particularly applicable to what is known in the art as continuous casting. In the art of continuous casting the supply of molten metal, either ferrous or non-ferrous, is continuously fed to one end of a mold cavity of suitable cross-section which is kept at a desirable temperature by a circulating fluid in contact with the outside of the mold wall and the cast metal withdrawn from the opposite end of the mold cavity without substantially interrupting the continuity of the ingot during the entire process. By means of continuous casting, ingots of a desired shape and of indefinite length and having superior properties may be cast in an economical and expeditious manner.

In the continuous casting of metal as described in United States Patent No. 2,079,644, issued May 20, 1937, to Edward R. Williams, a suitable method of and apparatus for continuous casting is described in detail. My invention is an improvement on the method therein described.

In casting continuous ingots by the process outlined in the Williams Patent No. 2,079,644, while generally satisfactory results have been obtained there is in some instances a tendency for the forming ingot to stick in the tube and for the ingot skin to rupture. This is probably caused either because the frictional resistance between the wall of the forming ingot and the mold wall is greater than the strength of the ingot skin or because the heat removed through the mold wall is not sufficient to produce a skin of sufficient thickness and strength to overcome any frictional resistance which may be present. It is also possible that, due to the fact that the ingot skin immediately starts to shrink away from the interior of the molding tube as soon as the metal is partly or wholly solidified, an air gap is formed between the ingot wall and the mold wall which insulates the ingot and reduces the heat transfer from the ingot to the mold wall. The molten metal inside the ingot skin would then deliver heat to the ingot skin which, because of the air gap and absence of direct contact with the mold wall, would not be transferred to the mold at a sufficiently rapid rate, and consequently the skin would be reheated and weakened to such an extent that it would rupture.

When rupture of the ingot skin occurs, the molten metal will escape through the opening and will immediately form a new skin when the metal comes in contact with the cold metal wall. This new skin has the appearance of a scab

because it does not become an integral part of the old skin. It is also thin and weak and ruptures again and again, thus causing the skin above it to remain stationary as the skin below it is pulled down. Unless this rupture is completely healed, it will continue to the bottom of the mold, at which point the molten metal will bleed completely out of the inside of the partly formed ingot above the rupture and the operation must then be stopped. It is also possible that, due to the formation of these scabs or rough spots, the diameter of the ingot is increased at this point and the increased diameter and roughened surfaces will so increase the friction between the formed ingot and the mold tube walls that more force is required to draw down the ingot than the ingot wall will stand. This may also be a contributing factor to the rupture of the ingot wall.

I have discovered that sticking of the ingot in the molding tube and rupture of the ingot skin can be avoided by coating the inner wall of the molding tube with a material which has a melting temperature much below the temperature of the formed ingot skin. For example, rolling mill lubricant may be applied to the inside of the molding tube. While one would expect that this would be almost instantly burned out, this is not the case because of the high rate at which the walls of the molding tube are cooled and also because of the limited amount of available oxygen, so that a small amount of lubricant will last an amazingly long time. Also, by having an oxidizable material on the wall of the molding tube, the limited amount of oxygen that may enter between the tube wall and the solidifying metal is consumed so that oxidation of the metal itself is avoided. It is not necessary, however, that the material be a readily oxidizable one as a slow oxidizing material or a non-oxidizable material may also be advantageously employed as a coating material to form a film.

The reason why the coating or film acts to facilitate the withdrawal of the ingots has not as yet been definitely ascertained. It may function:

As a thermal contactor to continue the heat transfer from the ingot to the mold wall when there is no perfect thermal contact between the outer wall of the ingot and the inner wall of the mold and enables a skin of sufficient thickness and strength to be formed to resist rupture during withdrawal. It is also quite possible that without some substance between the ingot wall and the mold wall, there never would be as nearly a perfect thermal contact (even at the point of

most intimate contact between the two) as when the film was added.

As a lubricant only—in which case it may function to reduce the frictional resistance between the skin of the ingot and the mold wall, and thus enable a thinner skin to be sufficient to resist the stresses incident to withdrawal.

As a plastic mold wall to produce a temporary wall of smaller diameter than the tube itself which, as the frictional resistance increases, can be squeezed out of the way and thus prevent sufficient frictional resistance to induce the rupture of the skin.

To prevent wetting of the walls of the molding tube or cooling cylinder by the formed ingot, thus reducing any tendency for adhesion or increase of frictional resistance between the ingot and the mold wall.

In the accompanying drawing there is represented a vertical section through a casting apparatus of the type to which the present invention pertains. The view illustrated corresponds to Figure 1 of the Williams Patent No. 2,079,644.

In the drawing, 15 represents a thin wall mold-  
25 ing tube of cylindrical form and fabricated from metal such as copper or brass having high thermal conductivity. The tube is open at both ends and is housed within a casing or jacket 16 in such a way as to provide a shallow cooling chamber 17 between the tube and the casing. A stool element 18 in the form of an ingot blank is located within and has a sliding fit with the tube 15. At the beginning of the pouring operation the blank is located at such a position within 35 the tube 15 as to provide a pouring cavity 19 at the top of the tube. Molten metal to be cast is delivered from the furnace by any suitable means such as a tiltable ladle 20 and is received by a pouring box 21 secured to the apparatus 40 adjacent to the top of the tube. The molten metal poured into cavity 19 is supported on the upper end of the ingot blank or stool 18 and bonded thereto by disconnectable lugs 22. In order to maintain a substantially constant tem-  
45 perature differential between the inner and outer surfaces of the molding tube 18 and to effectually remove the heat from the outer surface of the mold tube 15, a cooling medium such as water is introduced into the chamber 17 through 50 a pipe 23. The cooling water, after passing through the cooling chamber or jacket space 17 is discharged from the bottom thereof through the discharge pipe 24.

The lower end of the blank 18 is engaged by 55 suitable withdrawing mechanism having driven rollers 25 which contact the sides of the blank and also the sides of the ingot as it is being withdrawn. The rate of pouring and the rate of withdrawal of the unit are synchronized so that the 60 level of the metal in the molding tube will remain substantially constant. Heat is withdrawn from the metal at such a rate as to allow a skin to form which is sufficiently strong so that the ingot may be withdrawn without rupture of the 65 skin wall.

I have found that other lubricants beside oil and grease may be advantageously employed, for example, tri cresyl phosphate alone or mixed either with an oil or grease of high viscosity of 70 either mineral or vegetable origin. The lubricant preferably should have a fairly high boiling point and a fairly high viscosity. I have also found that by coating the interior of the mold

tube with a film of graphite, lead, solder or chrome, satisfactory results have been obtained in some instances.

While I have described a preferred embodiment of my invention, it will be understood that the invention may be otherwise practiced within the scope of the following claims.

I claim:

1. In the method of continuous casting of metal in a thin molding tube of high thermal conductivity cooled by a flowing thin sheet of fluid in contact with the outer walls of the tube, the step of maintaining on the inner wall of the tube a film of lubricating material having a melting point substantially lower than that of the metal being cast. 10

2. In the method of continuous casting of metal in a thin wall molding tube of high thermal conductivity cooled by a thin flowing sheet of fluid forced along and in contact with the outer 20 walls of the tube, the step of introducing on the inner wall of the tube and maintaining therealong for substantially the length of the tube a lubricant having a melting point substantially lower than that of the metal being poured. 25

3. In the method of continuous casting of metal in a thin-walled molding tube of high thermal conductivity cooled by a shallow sheet of fluid forced at high velocity along the outer walls of the tube, the step which consists of applying at 30 intervals to the molding surface of the tube and maintaining therealong for substantially the length of the tube a lubricating material which is fluid at a temperature substantially lower than that of the metal being poured. 35

4. In the method of continuous casting of metal in a thin-walled molding tube of high thermal conductivity cooled by a shallow sheet of fluid forced at high velocity along the outer walls of the tube, the step which consists of applying to 40 the molding surfaces of the tube in the vicinity of the metal being cast a lubricating material containing tri cresyl phosphate and maintaining said lubricating material in contact with the molding surface of the tube for a substantial proportion of the length of the tube. 45

5. In the method of continuous casting of metal in a thin-walled molding tube of high thermal conductivity cooled by a shallow sheet of fluid forced at high velocity along the outer walls of the tube, the step which consists of applying to 50 the molding surfaces of the tube in the vicinity of the metal being cast a lubricating material containing tri cresyl phosphate and a vegetable oil and maintaining said lubricating material in contact with the molding surface of the tube for a substantial proportion of the length of the tube. 55

6. The method of continuously casting metals of high heat content which comprises pouring the metal into a thin-walled molding tube of high thermal conductivity, scouring the exterior of the tube with a thin sheet of cooling fluid flowing at high velocity, withdrawing the metal from the opposite end of the tube after casting, introducing a lubricating fluid against 60 the side walls of the tube and keeping the inner surface of the tube sufficiently cool to maintain the lubricant along the interior of the tube throughout the operation and precluding the evaporation of such fluid before the pouring operation is substantially completed. 65

## DISCLAIMER

2,206,888.—*Charles T. Greenidge*, Columbus, Ohio. METHOD OF CONTINUOUS METAL CASTING. Patent dated July 9, 1940. Disclaimer filed March 3, 1942, by the assignees, *Edward R. Williams* and *Julia Lee Cox Williams*.

Hereby enter this disclaimer to claim 1 of said patent.

[*Official Gazette March 24, 1942.*]